

Dec. 14, 1937.

G. WEBER

2,102,245

EXPLOSIVE CHARGE AND APPARATUS FOR THE MANUFACTURE OF THE SAME

Filed May 26, 1934

2 Sheets-Sheet 1

*Fig. 1*



*Fig. 2*



*Fig. 3*



INVENTOR:

GUILLAUME WEBER

By: *Francis E. Bayce*

ATTORNEY

Dec. 14, 1937.

G. WEBER

2,102,245

EXPLOSIVE CHARGE AND APPARATUS FOR THE MANUFACTURE OF THE SAME

Filed May 26, 1934

2 Sheets-Sheet 2



INVENTOR:

GUILLAUME WEBER

BY: *Francis E. Boyce*  
ATTORNEY

## UNITED STATES PATENT OFFICE

2,102,245

EXPLOSIVE CHARGE AND APPARATUS FOR  
THE MANUFACTURE OF THE SAME

Guillaume Weber, Hayange, Moselle, France, assignor to Les Petits Fils de Francois de Wendel &amp; Cie, Paris, France

Application May 26, 1934, Serial No. 727,635  
In France June 17, 1933

5 Claims. (Cl. 102—5)

An explosive system is already known which consists of a certain quantity of water or of substances impregnated with water, and of a priming cartridge adapted to supply the heat necessary to cause the practically instant vaporization of the water.

On the other hand, a safety explosive is in use, which consists of solid carbon dioxide and a heating device, for example, a priming cartridge of any usual type, provided with a firing device, and the heat supplied by this cartridge causes the sublimation of the carbon dioxide.

The present invention has for its object an explosive which is chiefly characterized by the fact that it comprises a mixture of water snow and of carbon dioxide snow and a heating device adapted to vaporize said mixture.

Experience has shown that by utilizing together water in the form of snow, and carbon dioxide in the form of snow, it is possible to obtain effects which exceed those which have been obtained separately with the explosives above mentioned, due to the fact that the hot gases of the priming cartridge will penetrate more readily throughout the whole mass and will cause the instant vaporization and sublimation of the water snow and the carbon dioxide snow.

By the use of the combined cartridge containing water snow and carbon dioxide snow, the effect of the explosion lasts during a longer period of time, as the carbon dioxide is first sublimed, and the water snow is then vaporized. The effect of dislocation of ground is thus considerably increased.

On the other hand, all separate containers adapted to serve as a support for the water are eliminated, which results in a reduction of weight of the cartridge for a given force.

The water snow is preserved better according as the proportion of carbon dioxide snow, due to its temperature of  $-79^{\circ}$  C., is greater.

The proportion of water snow may vary, for instance, between 20 and 40%. As the carbon dioxide snow is sublimed before the water snow melts, the proportion of water snow increases gradually between the loading and the firing, and reaches about 50% at the time of firing.

Good results are already obtained with a proportion of water snow of 15 to 20%.

Obviously, instead of water, other substances which melt or vaporize at a temperature higher, for example, than the temperature of  $-79^{\circ}$  C. and which may produce a great volume of gas when heated at the time of the explosion, may

be utilized in the state of snow, in combination with the carbon dioxide snow.

The priming charge may consist of an explosive based upon liquid oxygen, or of any explosive, comprising the safety explosives. When provided with a safety explosive as the priming charge, the explosive system, water snow and carbon dioxide snow, may be proposed for coal mines containing fire damp and dust, and for potash mines containing fire damp.

In the accompanying drawings, which are given solely by way of example:

Figs. 1 to 3 represent, in longitudinal section, various methods of utilization of the explosive according to the invention.

Fig. 4 shows a diagrammatic vertical section of an installation adapted to be utilized for the manufacture of a mixture of water snow and carbon dioxide snow.

Fig. 5 is a partial section of the water injector.

The priming charge 22 with a detonator 23 is placed, at will, in front (Fig. 1), in the rear (Fig. 2) or at the middle (Fig. 3) of the charge of snow 25 and 25'. This latter is introduced into the mine chamber or hole 21, provided with a permeable casing 27, or more simply, without any protection, with resulting economy.

The packing 26 is carried out in the usual manner, and the firing is done by means of a cord or by electric conductors 24.

In order to obtain a mixture of water snow and carbon dioxide snow, the water snow may be produced at the same time as the carbon dioxide snow, by introducing into the receptacle 35 or expansion chamber of the carbon dioxide, water in a finely divided state, in the form of vapour or mist.

In the example shown in Figs. 4 and 5, the liquid carbon dioxide contained in the cylinders 40 1, such as are currently found in commerce, circulate through valves 2 and tubes 3 and expansion nozzles 4, into an expansion chamber 5 contained in a receptacle 6. In order to facilitate the formation of carbon dioxide snow by means of the expansion nozzles 4, the expansion chamber 5 is preferably surrounded by an envelope of wool 7. The receptacles 5 and 6 are provided with covers 8 and 9.

The installation further comprises a receptacle 50 10 containing water. This receptacle 10 is connected with a cylinder 11 containing carbon dioxide by a tube 12, provided with a valve 13. The water receptacle 10 carries at its upper part a pressure-gauge 14 adapted for the observation 55

- of the pressure of the carbon dioxide gas at the admission end of a tube 15 which is provided at the bottom with a sprayer 16 delivering into the expansion chamber 5. The water is supplied to the sprayer by a small tube 17 (Figures 4 and 5). The output of the water is greater or less according to the diameter of the orifice of the sprayer 16, which diameter may vary from a few tenths of a millimetre to a millimetre. Use is made, preferably, of carbon dioxide gas under pressure for spraying the water in order to be able, if necessary, to recover the carbon dioxide which is not solidified during the expansion, for further use, after passing through a gas-holder 18 into which it is circulated through the pipe 19 and from which it is again compressed in cylinders in view of another expansion. By this means, it is possible to reduce the loss of CO<sub>2</sub> to a minimum.
- 20 The covers 8 and 9 of the receptacle 6 and of the expansion chamber 5 permit the removal of the mixture of water snow and of carbon dioxide snow.
- 25 Obviously, the invention is not limited to the proportions, products and method of execution, described and represented, which are chosen solely by way of example.
- Having now described my invention what I claim as new and desire to secure by Letters Patent is:
- 30 1. A blasting charge comprising in combination a mixture of water in the form of snow and of carbon dioxide in the form of snow, and a heating element adjacent said mixture and adapted to produce the heat necessary to cause the instant vaporization of said mixture.
- 35 2. A blasting charge comprising in combination a mixture of carbon dioxide in the form of snow and of another substance in the form of snow adapted to be vaporized at a temperature higher than the temperature at which said carbon dioxide is sublimated, and a heating element adjacent said mixture and adapted to produce the heat

necessary to cause the instant vaporization of said mixture.

3. A blasting cartridge comprising in combination an envelope permeable to gas, in said envelope a mixture of carbon dioxide in the form of snow and of another substance in the form of snow adapted to be vaporized at a temperature higher than the temperature at which said carbon dioxide is sublimated, and a heating element adjacent said mixture and adapted to produce the heat necessary to cause the instant vaporization of said mixture.

4. A blasting charge comprising in combination a mixture of water in the form of snow and of another substance in the form of snow adapted to be vaporized at a temperature lower than 0° C., and a heating element adjacent said mixture and adapted to produce the heat necessary to cause the instant vaporization of said mixture.

5. An apparatus for preparing an explosive mixture of water and carbon dioxide in the form of snow comprising an expansion chamber, a container adapted to receive liquid carbon dioxide under pressure, communicating means between said expansion chamber and said container, a nozzle at the end of said communicating means situated in said expansion chamber, whereby liquid carbon dioxide is adapted to be introduced in a finely divided state from said container into said chamber, a receptacle adapted to contain gaseous carbon dioxide under pressure, conduit means between said receptacle and said expansion chamber, injecting means at the end of said conduit means situated in said expansion chamber, water supplying means, and guiding means between said water supplying means and said injecting means adapted to bring water from said supplying means into said injecting means, whereby said water is adapted to be introduced in a finely divided state by said gaseous carbon dioxide into said expansion chamber.

GUILLAUME WEBER.